

Jan. 24, 1950

2,495,396

J. URISON ET AL  
DESTRUCTIVE DISTILLATION OF VEGETABLE  
MATTER WITH CAUSTIC AND LIME  
Filed Oct. 30, 1945



## Inventors

J. Urisen

P. de Calignon

G. Pineard

G. Pingard  
C. F. Wenderoth  
Attorney

## UNITED STATES PATENT OFFICE

2,495,396

## DESTRUCTIVE DISTILLATION OF VEGETABLE MATTER WITH CAUSTIC AND LIME

Jacques Urisson, Paris, Philippe de Calignon, Lannemezan, and Gustave Pingard, Thann, France, assignors to Socete Pyreneenne de Carburants et Solvants, Paris, France, a French corporation

Application October 30, 1945, Serial No. 625,674  
In France October 19, 1944

Section 1, Public Law 690, August 8, 1946  
Patent expires October 19, 1964

2 Claims. (Cl. 202—34)

1

The present invention relates to the disintegration of celluloso-ligneous matters with a view to obtaining liquid condensable organic compounds consisting chiefly of products of ketonic character.

The drawing shows a flow sheet illustrating the steps of the method.

Our method comprises a preliminary impregnation, a heating in an autoclave and a pyrolysis treatment, these operations being carried out as follows:

Impregnation is carried out with a view to causing alkalis to penetrate into the pores, and especially into the capillary network of the matter to be treated, and obtaining a mass which is homogenous at the scale of the matter cut into small parts. This homogenizing of the impregnation obviously depends upon the nature of the raw material and the way in which it has been divided into small parts (by means of a straw cutter, a crusher, and so on), upon its dryness, the mechanical means used for mixing the whole, the temperature, and the pressure.

Impregnation must be carried out at a relatively low temperature, preferably averaging 50° C., at which temperature the vapor tensions inside the cells will oppose an admissible resistance to penetration of alkalis by dialysis. The important thing concerning this impregnation is to reach a homogenous state of distribution of the liquid in the solid material without allowing disincrustation, which corresponds to a reduction of the free or "active" alkali, to make substantial progress.

This impregnation must be carried out very carefully, and it is particularly delicate because the amount of liquid that is used is small with respect to the celluloso-ligneous material (from 0.7 to 3 litres of liquid per kilogram of wood).

The methods used for this impregnation and for checking the efficiency of the homogenizing are identical to those commonly used in wood impregnation industry. For instance we may use pressure, vacuum, both alternately (for elimination of the air that may be entrapped), or any other suitable means. However, in the present case, the particularly important thing is to avoid bringing the mixture to temperatures corresponding to a substantial disincrustation.

Heating is then carried out, for a relatively

short time (from 1 to 4 hours for instance), in an autoclave in which the temperature of the mass is raised to 160–180° C. in a very short time, for instance approximately from 10 to 15 minutes. In this way, we avoid keeping the mass for an appreciable time inside a zone of temperatures for which only the incrustant substances are solubilized, and we reach more rapidly the zone of temperatures for which cellulose itself is attacked, same as lignin, in suitable conditions and nearly simultaneously.

This quick rise of the temperature can be carried out only with a mass suitably impregnated with alkali. Otherwise, that is to say in the case of a heterogeneous mixture, exothermic phenomena take place, with a production of gases and even a spontaneous degradation of the celluloso-ligneous matter analogous to carbonization.

This heating may be carried out with the apparatus commonly used in the manufacture of paper pulp through the soda process, and the quick rise of temperature may be obtained, under industrial conditions, by an injection of steam into the autoclave.

After heating, lime, either slaked or unslaked, is added to the mass and the whole is dried, preferably at a temperature of 160–180° C., this temperature being maintained for some hours after the drying is completed. This prolonged drying treatment serves to produce a deeper degradation of the celluloso-ligneous matters, characterized by a reduction of the active alkalinity and of the proportion of organic substances that are not scoured.

The uncondensable gases and the vapors that disengage during the heating and drying treatments, and also the uncondensable gases resulting from the pyrolysis treatment, may be used advantageously for sweeping or scavenging the free space of the pyrolysis apparatus, instead of using for this operation steam produced especially for this purpose as in known pyrolysis treatments.

This supplementary production of steam is thus avoided or at least greatly reduced and, on the other hand, dilution of the products that are obtained, as a result of the condensation of said steam, is avoided.

We will now describe two examples of the method according to our invention:

2

## 3

## Example I

The following elements are intimately mixed together:

100 kgs. of oak saw-dust  
60 kgs. of caustic soda  
60 kgs. of water.

Caustic soda is used under any physical form whatever. Water is introduced partly in admixture with wood and soda, and the amount of water necessary to give the above indicated amounts is added. The mass is left alone for 12 hours for impregnation purposes.

The whole is then introduced into a rotary autoclave of a capacity of 450 litres, externally heated. The temperature is brought to 180° C. in a quarter of an hour and this temperature is maintained for 3 hours. The apparatus is then placed in communication with a vapor accumulator or with the pyrolysis apparatus and the pressure is allowed to drop to a value approximating atmospheric pressure. The mixture of organic salts that is obtained still contains at this time about 12 percent of organic substances not scoured, with respect to the starting material.

120 kgs. of slaked lime are added and the temperature is again brought to 180° C. This temperature is maintained for 2 hours, while expanding the vapor into the vapor accumulator.

After this drying treatment, the mixture contains only 8 per cent of organic substances not scoured.

The whole is pyrolysed in a rotary furnace, of the continuous working type, heated from the outside (outlet temperature ranging from 500 to 600° C.). The apparatus is swept by a stream of steam and vapors resulting from the heating and drying treatments.

After condensation, 21 kgs. of liquid valuable products are collected, the weights corresponding to anhydrous products, to wit:

|                                        | Kgs. |
|----------------------------------------|------|
| Acetone+methyl alcohol                 | 5    |
| Light oils (flash point below 220° C.) | 9    |
| Heavy oils (flash point above 220° C.) | 7    |

If the drying operation is dispensed with, only from 10 to 15 kgs. of products are obtained.

## Example II

The following elements are intimately mixed together:

100 kgs. of vine-shoots,  
50 kgs. of soda,  
36 kgs. of water.

The mixing is pursued, at a temperature of 70° C., in a rotary apparatus, for 2 hours. The mass is then introduced into a rotary autoclave. The temperature is raised to 170° C. in ten minutes, by introduction of live steam, and this temperature is maintained for two hours. The pressure is then allowed to drop to a value substantially equal to atmospheric pressure, by elimination of steam.

The proportion of unscoured organic substances in the mass is then about 20 per cent of the initial matter.

125 kgs. of unslaked lime are then added and the temperature is brought to 180°, by external heating. This temperature is maintained for 2 hours and the pressure is caused to drop by elimi-

## 4

nation of steam. The proportion of unscoured organic substances drops to 4 per cent after this drying treatment.

The mass is introduced into a pyrolysis furnace 5 and the temperature is gradually brought to 600° C., with a sweeping of the furnace by the gases and vapors produced by the heating and drying operations above referred to. We obtain, after condensation, 22 kgs. of liquid products of value, 10 containing:

|                                        | Kgs. |
|----------------------------------------|------|
| Acetone+methyl alcohol                 | 6    |
| Light oils (flash point below 220° C.) | 8.5  |
| Heavy oils (flash point above 220° C.) | 7.5  |

15 These treatments are given merely by way of example and they may be modified, both concerning the operations in themselves and the particular bodies that are used, without departing from the spirit of the invention.

20 The final residual mass, after pyrolysis, is constituted by sodium and calcium carbonates, soda, lime, and a residual carbon containing a percentage of hydrogen which depends upon the final pyrolysis temperature. This residue may be treated according to the known methods for caustification of the amount of  $CO_3Na_2$  present in the soda lye.

25 The mixture of calcium carbonate and coal is then calcined, the residual coal adding itself to the fuel that is supplied. The calcium carbonate is transformed into unslacked lime for being returned into the cycle of operations.

30 The whole of the reagents that have been employed can thus be returned into the cycle with the exception of course of the losses due to the operations.

35 It is also possible to recuperate the residual coal and to utilize it as activated coal for instance. 40 This activity depends upon the proportion of hydrogen present therein and the final pyrolysis temperature.

45 In a general manner, while we have, in the above description, disclosed what we deem to be practical and efficient embodiments of the present invention, it should be well understood that we do not wish to be limited thereto as there might be changes made therein without departing from the principle of the present invention as 50 comprehended within the scope of the appended claims.

What we claim is:

1. A method of producing liquid condensable 55 organic compounds from vegetable cellulosic material, which comprises impregnating this cellulosic material with a caustic soda lye at a temperature relatively low, treating the impregnated material in an autoclave in the presence of caustic alkali by quickly raising the temperature of 60 the mass up to 160-180° C., adding lime to the mass, drying at a temperature of 160-180° C., keeping said mass at this temperature for several hours after the end of the drying operation, and treating by pyrolysis.

65 2. A method of producing liquid condensable organic compounds from vegetable cellulosic material, which comprises impregnating this cellulosic material with a caustic soda lye, at a temperature of approximately 50° C., treating the impregnated material in an autoclave in the presence of caustic alkali by raising the temperature of the mass up to 160-180° C. in 10 to 15 minutes, by injection of live steam into the autoclave, adding lime to the mass, drying at a temperature of 70 160-180° C., keeping said mass at this tempera-

ture for several hours after the end of the drying operation, and treating by pyrolysis.

JACQUES URISON.

PHILIPPE DE CALIGNON.

GUSTAVE PINGARD.

**REFERENCES CITED**

The following references are of record in the file of this patent:

**UNITED STATES PATENTS**

| Number    | Name   | Date          |
|-----------|--------|---------------|
| 1,202,479 | Rinman | Oct. 24, 1916 |

| Number      | Name      | Date           |
|-------------|-----------|----------------|
| 1,298,479   | Drewson   | Mar. 25, 1918  |
| 1,764,249   | Erlenbach | June 17, 1930  |
| 1,772,216   | Hagglund  | Aug. 5, 1930   |
| 5 1,879,502 | Rinman    | Sept. 27, 1932 |
| 2,177,557   | Bergstrom | Oct. 24, 1939  |
| 2,056,746   | Strupp    | Oct. 6, 1946   |

**FOREIGN PATENTS**

| 10 Number | Country       | Date          |
|-----------|---------------|---------------|
| 114,878   | Australia     | Mar. 11, 1942 |
| 424,847   | Great Britain | Mar. 1, 1935  |